

## UNITED STATES PATENT OFFICE.

ROBERT FULTON TOMPKINS, OF NEW YORK, N. Y.

BINDING AND COHERING COMPOSITION.

Div. of 1171905

1,247,595.

Specification of Letters Patent. Patented Nov. 20, 1917.

No Drawing. Original application filed August 11, 1913, Serial No. 784,121. Divided and this application filed February 11, 1916. Serial No. 77,599.

*To all whom it may concern:*

Be it known that I, ROBERT FULTON TOMPKINS, a citizen of the United States, residing at New York, in the county of New York and State of New York, have invented certain new and useful Improvements in Binding and Cohering Compositions, of which the following is a specification, being a division of Serial No. 784,121, filed August 11, 1913.

This invention relates to binding compositions for substances of divided or separated nature, such as sand or insoluble silicious or silicon containing material, or other substances of mineral, vegetable, or animal nature, and process of making same.

The object of the invention is to provide an efficient binder of vegetable nature or a carbon compound character comprising a glucosid, or tannin and glucosid associated with water, or water and soluble silicates, such as sodium silicate and has for certain specific applications the property of binding, securing or anchoring road-dust together in such a manner that its circulation by air currents occasioned by moving vehicles or other means is limited or prevented and whereby a solid compact and hardened road-bed and road dressing is produced and an automatic hygroscopic coherence or adherence created, without materially injuring or destroying the coherer or adhering binder, and also for binding molder's sand or compositions for cores, etc., for gluing, sizing, or cementing of cellular or cellulose containing material or products or fabrications thereof, such as paper, paste-board, straw board, and the like, and for other purposes.

One species of the composition included in the present invention comprises glucosids of the aromatic extractives type, such as glucosid tannins which appear in tanning extracts or products, in proportion of about 27% by weight together with tannin 21% and water 52%, which composition has an approximate gravity of forty-eight degrees Twaddell.

This product or composition may be produced by concentrating the spent tan liquors containing approximately 2% of glucosid and tannin in approximate pro rata proportion to each other by weight as one and a half to one, or an aqueous solution of 2%

Twaddell, by evaporation or hydration to a density of 48 degrees Twaddell.

To this aqueous solution of glucosid on tannin is preferably added a soluble silicate such as sodium silicate, in proportion of 5% by weight of the combined glucosid and tannin content when the binder is intended to be employed as a street or road dressing or as a cement or glue for paper, straw, or other cellulose containing substances or fabrications.

The advantages of this binder, comprising glucosids and tannins resides in the fact that when applied to paper or other cellulose substances which are matted or bonded by glues or sizes of glue nature, that the glucosid tannins and other tannins act as a glue or binder while they simultaneously fix the glue or size bonding material in the paper or other cellulose fabrication making a practically water repelling seal or binding, while the glucosid present is just sufficiently hygroscopic to prevent the drying out of the material to a point of brittleness thus producing a substantially water-repellent and flexible or resilient gluing medium. The soluble sodium silicate, when employed, also augments the adhering of the composition and maintains a flexibility which does not occur when substances comprising the silicate alone, as in the prior art, are employed.

When the binder is employed as a road dressing or binder, the tannin or tannic acid combines with the iron, alumina, lime or other constituents of the road construction material producing water insoluble compounds which present to the glucosids and other ingredients of the binder a superior adhesive surface so that the glucosids and excess tannins act as an agglutinating agent for anchoring or securing particles of dust or other material together in a fixed and flexible or elastic manner while the inherent hygroscopic properties of the glucosids provide a ready and automatic moistening constituent and effect without deliquescence so that the particles adhere together without becoming attached to foreign materials which may contact with them such as vehicle tires, etc.

The glucosids employed may be of any selective character, they being compounds which combine the properties of glucose and vegetable extractives, or what may be termed

glucose esters, in such a manner that each has lost its specific physical identity as such and is less soluble than either individually in water as a rule, and is hygroscopic without deliquescence and does not effloresce or dry up spontaneously. The peculiarly adaptable properties or qualities of these glucosids probably is attributable to a progressive and alternate hydrolysis into vegetable extractives or organic or carbon containing acids and glucose and its reformation of glucosids by condensation and dehydration under atmospheric conditions of heat, moisture, and pressure.

15 The soluble silicate, such as sodium silicate, augments the cementing and anchoring qualities of the composition especially when associated with insoluble silicates, silicious, or silicon containing substances such as are 20 usually found associated with or form a part of road construction.

25 The composite composition of these ingredients associated with water therefore produces a peculiarly advantageous material of selective utility as a cement or binder of flexible resilient, and elastic nature in character.

30 Any glucosid associated with tannin may be employed and mixed in any selective or desired proportion without departing from the spirit of the invention, so long as both are present in some form or the glucosid in itself presents and exhibits the combined properties hereinbefore set forth.

35 The soluble silicate, such as sodium silicate, may be employed as a binder augmenting agent or additive constituent of the composition to modify the properties thereof with reference to its silicious cementing 40 character and also for the purpose of resinifying some of the tannins and converting them into more water repellent substances.

45 The composition of tannin and glucosids may be produced by mixing the individual ingredients with water or secured from such substances as spent tan liquors, or from other sources, or extracted from natural derivatives, or artificially or synthetically prepared.

50 Some of the tannins and tannic acids are at once so called tannins and glucosids, they being converted by hydrolysis into glucose and gallic, ellagic, protocatchuic and other acids or organic extractives.

55 The composition comprising glucosids and tannins together with water, such as may be obtained from or as spent tan liquors, or fluid tan waste products such as are ordinarily thrown away, either as such or products which may be obtained by boiling down or concentrating the same, or such concentrated product rediluted, is particularly adaptable to road treatment, acting as it does to fix the dust and cement the road base 60 thus maintaining a form of fixed binder

which is continually working its way into and between particles or pieces of the road construction when subjected at intervals to progressive watering either by artificial sprinkling or from the natural source of 70 rain, etc., and exhibits the further enhancing quality of presenting a latent form of moisture by reason of its hygroscopic properties thus preventing the disintegration and drying out or crumbling of the road dressing 75 or base body and also provides a superior dressing or binding agent for construction materials of roads or other solid vehicle or transportation bearing body or path.

This material applied to the surface of 80 such roads as asphalt roads or pathways, and then coated or sanded with frictionable substances, has the property of anchoring or securing such material to the asphalt surface thereby preventing the slipping of 85 horses or skidding of vehicle wheels, the astringent properties of the tannin ingredients augmenting the frictional surface of the road as presented to contacting substances such as vehicle tires, and also present the 90 additional feature of holding and securing or anchoring frost and ice to the roadway in such a manner that it is not easily released under pressure and forms a foothold of frictional character for horses' shoes and the 95 like, thus avoiding the usual dangerous character presented when ice is formed upon water repellent surfaces such as asphalt, which results in slipping under pressure through the release of the unanchored ice 100 coating.

The preferred process whereby this composition is made for employment as a road or roadway dressing, is to secure or provide a spent tan liquor from a tannery or other 105 source which averages in density approximately two degrees Twaddell or about two per cent. of soluble content comprising tannin and glucosids in proportion of about one of the former to one and a half of the latter 110 by weight; this spent tan liquor is then exposed to the action of heat either by direct means or through the medium of circulating air at a higher temperature than the liquor and preferably under reduced pressure 115 whereby the vaporization of the aqueous content or evaporation of the material is facilitated. This drying or dehydrating action is continued until the fluid or liquor has been concentrated to about forty eight degrees 120 Twaddell or approximately 48% of the tannin and glucosid. This concentration to 48 degrees Twaddell is made in order to facilitate the preservation of the liquor from decomposition and to cheapen and facilitate 125 shipment to points where it is to be utilized. This concentrated liquor is then diluted with water in the locality where it is to be employed in proportion of one part of concentrated liquor to three parts of water for 130

a first coating or sprinkling of a road or roadway and one part to two parts of water for a second or final coating or sprinkling.

This dust cohering and roadway cementing fluid has the advantage over oil dressings in that it does not injure or destroy rubber tires or vehicles or affect the varnish of the same injuriously, nor is it lost by evaporation, or does it affect injuriously metal, wood or leather, or reduce the gravity of the road dressing so that it is floated and washed away by water or give a greasy appearance or dull coating to varnish or contents of vehicles.

Having now described my invention what I claim as new and desire to secure by Letters Patent, is:—

1. A cohering or binding composition comprising a hygroscopic glucosid, and a soluble silicate.
2. A cohering or binding composition comprising a hygroscopic glucosid, a soluble silicate and water.
3. A cohering or binding composition

comprising a hygroscopic glucosid and 25 sodium silicate.

4. A cohering or binding composition comprising a hygroscopic glucosid, sodium silicate and water.

5. A cohering or binding composition 30 comprising a carbonaceous extractive constituent of tan bark liquor containing a hygroscopic glucosid.

6. A cohering or binding composition comprising a carbonaceous extractive constituent of tan bark liquor containing a 35 hygroscopic glucosid and a soluble silicate.

7. A cohering or binding composition comprising a carbonaceous extractive constituent of tan bark liquor containing a 40 hygroscopic glucosid and sodium silicate.

In testimony whereof I affix my signature in the presence of two witnesses.

ROBERT FULTON TOMPKINS. [L. S.]

Witnesses:

F. L. WHOITNER,  
ERNEST H. BALL.

Copies of this patent may be obtained for five cents each, by addressing the "Commissioner of Patents, Washington, D. C."